

## UNITED STATES PATENT OFFICE

2,351,811

## PROCESS OF PREPARING FRITTED FOUNDATIONS FOR THE ENAMELING OF METALLIC ARTICLES

Karl Frank, Bad Soden in Taunus, Germany;  
vested in the Alien Property CustodianNo Drawing. Application April 19, 1938, Serial  
No. 202,907. In Germany April 22, 1937

2 Claims. (Cl. 204—38)

The present invention relates to a process of preparing a fritted foundation for the enameling of metallic articles.

The best adhesion between iron and enamel has hitherto been obtained by the use of a fused foundation containing an adhering oxide. This process is chiefly used in the case of wrought-iron and for small pieces. In the case of cast iron the top enamel powder has to be applied to the fused foundation in the hot condition which, of course, is only possible with small objects; large pieces radiate too much heat.

When a fused foundation is used, the resistance of the enameled objects to sudden temperature changes is, however, relatively small. As soon as such an enamel is quenched with ice-water from a temperature of 90° C. it shows capillary cracks. Enameled objects of wrought-iron are somewhat less sensitive than enameled cast iron objects, owing to the adhering oxides, but even their resistance to sudden temperature changes is generally unsatisfactory in practice.

If instead of a fused foundation a fritted foundation is used, the resistance to sudden temperature changes of the enamel may be increased considerably. The adhesion between the fritted enamel and the iron, however, is considerably smaller than that of an enamel with a fused foundation so that more or less large pieces of enamel break away from the coating without any visible reason, whereby the objects become useless.

Attempts have been made to improve the adhesion of fritted enamels, and of enamels in general, by roughening the metal surface, especially iron, either by a mechanical treatment, for instance by a prolonged blast of quartz sand or steel sand, or by a suitable pickling. The sand blast attacks the soft constituents more than the hard constituents, for instance the cementite, so that later when the enamel is fired a disintegration and loosening of the enamel may set in where the cementite crystals are situated. When pickling is used it is inevitable that removal of iron by dissolution leaves carbon at the surface, for instance in the form of graphite; this also entails a defective enameling.

Now I have found that a fritted foundation may be prepared without the drawbacks named above. According to the invention the metal surface is roughened, not as hitherto usual by removing the soft constituents by chemical or mechanical method, but by applying a new metal layer on the metal surface to be enameled, preferably freed from oxide in the usual manner.

The new metal layer is applied in such a manner that as rough a surface as possible is obtained.

For applying the metallic intermediate layer there exist various possibilities. The metal to be applied may, for instance, be heated to a high temperature and then applied by spraying. Care must be taken by suitably guiding the flame and, if desired, by using a protecting gas that on the one hand an oxidation of the metals and on the other hand an undesired absorption of hydrogen, carbon and the like is avoided. Furthermore, the spraying device must be constructed in such a manner that a coating as rough as possible but of good adhesion is obtained.

15 Another method for applying a metallic intermediate layer on the metal surface consists in depositing metal from liquid or gaseous metal compounds. For this purpose there are preferably used carbonyls, for instance for enamels on iron the carbonyls of iron or of nickel. These carbonyls are suitably decomposed under a reduced pressure at a raised temperature, for instance between 120° C. and 200° C. It is advisable to choose such a temperature for producing these deposits that the carbonyls will not decompose in contact with any ceramic substances or the like which may be present but only with the iron surface owing to the metallic action of the iron. Especially suitable temperatures for iron carbonyls are those below 180° C. The temperature and also the pressure and the other conditions, however, may vary according to the desired roughness of the coating or to the presence of small quantities of a protective gas. Instead of decomposing carbonyls the metal may be applied by decomposing other metal compounds, for instance by a reduction of a metal halide or the like.

40 A third method of applying a metallic intermediate layer is the galvanic separation of a metal on the object to be enameled. In this procedure the electrolysis is conducted in such a manner that the deposit is as coarse-grained as possible. This may be attained by a high amperage. At the same time any hydrogen discharge should be avoided as far as possible, for instance by continuously moving the electrolyte or by heating.

45 For iron objects deposition of iron or nickel by one of the aforesaid methods is preferable.

The rough metallic layer may be deposited either directly on the quite clean metal which for this purpose has been freed from rust, for instance by pickling, or by a mechanical treatment, or through a porous intermediate layer

which previously has been fritted or even through a porous non-fritted layer resistant to water and acid which may subsequently be fritted.

It is possible, for instance, first to apply by a usual method a fritted porous layer on the objects to be enameled. Such a fritted layer may consist, for instance, of about 70 per cent. of silica, the residual 30 per cent. comprising alkalies, boric acid, lime and some alumina. In this fritted layer the content of silica is so high that the fritting does not lead to complete dissolution in the fluxing material but only to a fritted but still relatively porous mass. This porous mass adheres to the iron surface, it being possible, owing to an oxidation of the surface of the iron, that an intermediate layer of iron silicate or the like is present. Owing to the porosity of the fritted layer it is now possible to deposit a metal or the iron surface, by the use of carbonyls or galvanically, through the fritted layer and so to obtain a rough surface. If necessary, the material must be pickled carefully before this deposition of metal in order to expose clean metal in the pores of the fritted base. The applied metal fills the pores and an especially intimate connection and interlocking of the metal and the fritted layer is produced. This connection is so intimate that it is very difficult to remove the fritted layer or a top enamel applied thereon, so that detachment of large pieces is impossible.

If the layer through which the metal is to be deposited is to be a non-fritted layer, the procedure is similar to that applied in the known manufacture of acid-proof self-hardening water glass cements, for instance by admixture of small proportions of such substances as cause the mass to harden even in absence of air. For instance, a mixture of 100 grams of a frit basis having a high content of quartz, consisting of quartz powder and a frit containing alkali not too finely pulverized, with 4 grams of potassium silicofluoride and 30 cc. of potassium water glass is stirred together with 40 cc. of water so as to form a slip which is then applied on the iron surface by a known method, for instance by spraying or casting. After some time the mass hardens by itself and becomes acid-proof and water-proof. Metal may now be deposited, for instance galvanically through the pores of this coating. One or more top layers of enamel are then applied and the object is fired.

In this operation the following drawback is sometimes observed: The layer of the frit basis cemented by water glass contains, after the hardening, silicic acid gel which during the galvanic deposition of metal absorbs small quantities of the metal salt used in the electrolysis, for instance metal chloride or metal sulfate. If after the electrolysis top enamel is applied on the fritted layer and dried and fired, the metal salt decomposes at the high temperature and bubbles and pores are formed.

It is possible to remove this drawback by treating the frit layer after the metal has been deposited with a solution containing such cations which react with the anions of the solution of metal salt used for the electrolysis and form compounds which at the firing temperature subsequently applied do not decompose with evolution of gas.

If, for instance, through the frit layer cemented with water glass iron is applied by the electrolysis of iron chloride solution the treatment must be with a solution containing cations that form chlorides which still do not decompose at about

800° C. with evolution of hydrogen chloride. The most suitable solution of this kind is baryta water which reacts with iron chloride with formation of ferric hydroxide and barium chloride. The barium chloride does not melt below 960° C., that is it melts at a temperature above the firing temperature of the top enamel. The barium hydroxide solution for the treatment of the fritted base is preferably used in a concentration of 1 to 5 per cent.

The layer of frit containing water glass may best be applied by spraying. This operation, however, has the drawback that during the spraying a relatively large quantity of the foundation frit is lost.

This drawback may be avoided if the foundation frit is applied by pouring or spraying it, as usual, on the metal surface without previous admixture of water glass, and then fixing it. The fixing is preferably performed by spraying on water glass solution together with an addition which causes self-hardening of the water glass, for instance a silicofluoride. It may be advisable, before spraying on the water glass, to dry somewhat the cast layer of foundation frit.

The foundation frit may be poured or sprayed on either merely suspended in water or with an addition of any usual organic or inorganic binding agent.

It is also possible to add the self-hardening agent to the foundation frit suspension itself and after the layer has been dried to spray on water glass solution. In this case the binding of the water glass with the foundation frit occurs by itself.

There may also be used materials other than water glass for fixing the foundation frit if they combine the particles of the frit with each other and with the metallic surface in a manner so porous and so stable that separation does not occur during the subsequent treatment in the galvanic bath.

For the application of the valuable foundation frit casting is particularly suitable for in this case there are practically no losses of the suspension and the water content of the latter may be adjusted as desired to suit other conditions without the danger of formation of cracks.

Similar coatings stable to acid and water may also be produced by any desired other process, for instance by mixing the foundation frit named above in the form of a fine powder with a combustible binding agent which is insoluble in water, for instance with varnish lacquer, and applying it on the object to be enameled by spraying. In this case the impinging drops of varnish lacquer and frit form a porous layer consisting of single globules on the metal surface, through which porous layer metal is deposited whereby an intimate connection of the frit and the metal, even during the firing, is attained.

By this new process it is possible to produce a fritted layer which leads to an extraordinarily good adhesion of the top enamel, if necessary also of any intermediate enamel layers between the frit layer and the top enamel, with a very high resistance of the whole enameling to sudden variation of temperature.

I claim:

1. The process of preparing a metal article to receive a fused enamel coating which consists in first applying a porous waterproof and acidproof fritted foundation to the surface of the article and thereafter galvanically depositing a bonding

metal upon the said metal surface through the pores of the fritted foundation.

2. In the process of preparing a fritted foundation for subsequently applying enamel on metallic articles by firing, the step which comprises galvanically depositing a metal on the metal surface through the pores of a water-proof

and acid-proof porous non-fired layer applied on the metal surface and substantially consisting of fritted foundation with an addition of water glass and an alkali metal silicofluoride which causes the mass to harden in the absence of air.

KARL FRANK.